

## UNITED STATES PATENT OFFICE

2,117,856

METHOD OF PRODUCING IRON CORES FOR  
ELECTROMAGNETIC COILSWilhelm Scheppmann, Berlin-NeuTempelhof,  
Germany, assignor to C. Lorenz Aktiengesell-  
schaft, Berlin-Tempelhof, Germany, a com-  
panyNo Drawing. Application July 11, 1935, Serial  
No. 30,917. In Germany July 14, 1934

2 Claims. (Cl. 175--21)

It is well known to produce the iron cores for electromagnetic coils, especially those for self-induction coils intended for high frequency purposes, of a finely divided iron powder. To such end a powder of this nature is embedded in an insulating material that acts to separate the iron particles from each other. The powder in this state is compressed to form a core of the desired shape.

10 The invention relates to methods of producing such cores of this type as are intended for high frequency circuits. It is proposed by the invention to make use of amber in producing an insulating material adapted for the said purpose. In this way the property of the amber is utilized that it is a material of small dielectric losses.

The novel method is as follows.

The known iron powder is mixed with a solution of amber not too viscid. After mixing, which 20 must be made very carefully in order to obtain

a substance as homogeneous as possible, the powder is dried. Each iron particle has thus been coated with a thin layer of amber. The powder when dry is, before getting compressed to form the core, moistened with some turpentine oil in order that the compressed material be given a greater mechanical solidity.

The usual pressures are employed in accomplishing the compressing action.

What is claimed is:

1. A method of producing iron cores for high frequency electromagnetic coils, characterized by combining iron powder with an insulating material consisting essentially of amber.

2. A method of producing iron cores for high frequency electromagnetic coils which consists in mixing iron powder with a solution of amber, drying this mixture and compressing it to form the core.

WILHELM SCHEPPMANN. 20